

## UNITED STATES PATENT OFFICE.

CHARLTON WILDER, OF CINCINNATI, OHIO, ASSIGNOR TO THE CROWN ROCK ASPHALT COMPANY, OF CINCINNATI, OHIO, A CORPORATION OF OHIO.

## PROCESS OF MAKING ROADS.

No Drawing.

Application filed June 29, 1925. Serial No. 40,451.

My invention relates to a process of preparing, shipping and laying rock asphalt.

The invention herein described is adapted to be practiced on any rock asphalt, but the times, temperatures and other conditions are disclosed herein with particular reference to the treatment of rock asphalt from Grayson County, Kentucky. This asphalt averages approximately 5.65 percent bitumen and the mineral aggregate is sharp, hard and graded sand analyzing 98.27 percent silica. There is also present from  $\frac{1}{2}$  to  $\frac{3}{4}$  of one percent moisture.

There is very little exact or dependable chemical information concerning bituminous substances and particularly rock asphalt. Asphalts are supposed to be of petrolic origin and contain a great variety of hydrocarbons of numerous different series and a wide range of molecular weights. Some of these hydrocarbons are aliphatic, some aromatic, some saturated and some unsaturated. The bituminous content of natural rock asphalt is supposed to differ from that of asphalt such as Trinidad Lake asphalt, in that more unsaturated hydrocarbons are present. Because of this paucity of exact information the chemical or physical actions and reactions which either take place or are prevented by this particular process can only be expressed by reference to their manifestations, that is, by the change in color or physical condition of the product which has been found to be critically significant in many cases including the present instance. When the rock asphalt is mined it is of a gray or brown color, or gray brown color. The particles of the rock asphalt do not adhere readily together just after being mined and the material can be handled with a shovel or with other ordinary implements. After it has been placed on the road however and subjected to the action of the sunlight which seems to be peculiarly catalytic in effect, the gray or brown, or gray brown color changes to a bright black. The particles of material then adhere securely together. Otherwise expressed, the material seems to set up as it changes color. In this latter condition the asphalt is very hard and cannot be readily handled or shipped.

It is desirable for road building purposes

that the asphalt used contain approximately 7 percent bitumen. In order to meet these requirements it is necessary either to discard a large percentage of the rock asphalt mined, or to fortify it with additional asphalt or bitumen.

A suitable bituminous fortifying agent is Trinidad Lake asphalt. From 8 to 10 percent in quantity of Trinidad Lake asphalt is cut back with the oil flux of an asphaltic base petroleum, said oil flux having a penetration of from 300 to 350. However, any asphaltic or bituminous material can be used, the advantage of the Trinidad being that it has incorporated therewith colloidal dust and is otherwise of hard quality adapted to raise the general average hardness of the bitumen of the resulting product.

In view of the soft nature of the bitumen of the rock asphalt, this fortifying with a harder grade is often desirable. However, it has generally been regarded as impossible to get a hard grade of bitumen or in fact anything other than an oil to mix with the rock asphalt as mined, without the application of heat to make it more fluid.

Heretofore it has been considered essential, indeed it was the invariable practice in the art, to either employ such relatively high temperatures in connection with the mixing treatment, or else to continue the heat application during the mixing to a point where the asphaltic rock changed from its gray or gray brown color characteristic of the crude mined product to the bright black color characteristic of the finished or ultimate product. In consequence of this completion of the cooking incidental to the mixing operation as heretofore carried on in practice, the asphaltic rock reached the "set up" or hard agglomerate and solidified mass condition at the completion of the mixing stage and this refractory material necessarily had to be physically or mechanically reduced or broken up at a great expense and with some loss in order to restore the set up material to the loose or fluctuant physical state suitable for shipment manipulation or for road application. This economic waste and physical disadvantage has been a long recognized and familiar problem in the art, which has heretofore been regarded as inherent in and inevitably

incident to the nature of the material when subjected to the requisite mixing and heat treating operations.

Attempts have been made to render the 5 set up rock asphalt shipable by mixing with it a quantity of volatile oil adapted to take away the rock-like properties of the mass. In theory the volatile oil evaporates after the rock asphalt is laid but in practice it does not entirely disappear, particularly from the base of the road. Consequently rock asphalt so prepared for shipment produces roads of inferior strength and quality accompanied by a very undesirable 10 road mobility.

My process supplies a definite and satisfactory solution of this difficulty in providing a suitably fortified asphaltic rock which at the end of the mixing stage is in a 20 physical state and condition most advantageous for handling, shipping and manipulation, by reason of its meal-like relatively pulverulent mass, or unset-up state. In other words, the material produced by my 25 process is in effect a new material in the industrial or economical sense, i. e., a raw but fortified, unset-up asphaltic rock existing in a more or less disintegrated physical state suitable for both shipment and road 30 application manipulations. This raw or unconditioned material is converted from this state to its finished product or set-up state either by secondary heat treatment after shipment or by sun exposure after road 35 application.

The object of my invention is to provide a process for making roads of hard uniform quality and up to specifications out of natural rock asphalt, the bituminous content 40 of which is below specifications.

Another object of my invention is to provide a process for fortifying natural rock asphalt with additional asphaltic or bituminous binder without impairing the characteristics of the material from the view 45 point of shipping the same.

After the natural rock asphalt is mined it is ground up into a rock meal of such fineness that most of it will pass through 50 a quarter inch screen. A hammer reducing mill is very suitable for this operation. Next, samples are taken to determine the exact bituminous content of the rock meal in order to calculate how much it must be fortified. The material is then passed into a 55 revolving drum heated by an oil burner where it is kept, for approximately two minutes. It emerges from this drum at a temperature of 100° to 150° F. It is next 60 put into a mixer where the bituminous fortifying element is added. The mixer is preferably of the double shaft and paddle type. The fortifying bitumen is introduced 65 at a temperature of from 200 to 250° F., and 70 the entire mass is mixed from one to two

minutes. The 100° to 150° of temperature of the rock asphalt is not sufficient to cause the change chemical or physical which is manifested by the change of color and the setting up of the mass, yet the temperature 75 is sufficient to prevent undue chilling of the fortifying bitumen which is introduced. The temperature of from 200° to 250° is adequate to make the fortifying bitumen sufficiently fluid to mix readily, but the percentage of bitumen being in the neighborhood of two percent of the total mass, at the most, is not sufficient in quantity to raise the temperature of the entire mass to such a degree that the rock asphalt changes color 80 and condition.

After this mixing operation, the resulting material is placed in storage piles. It can be handled with shovels and by ordinary methods for shipping, and does not need to 85 be dynamited out of the storage pile as would be necessary had the color changed. After shipment it is laid cold upon the road and raked and rolled in the usual manner. It should preferably be laid in warm dry 90 weather and the sun's heat and light is sufficient to cause the laid rock asphalt to change color, set up and form into a solid mass right on the road. Rock asphalt usually continues this setting up process over 95 some period of time—often two or three years. A partial change is advisable before opening the road to traffic. This partial change or setting up should preferably take place before rolling and the greater its degree the less danger will there be of early 100 traffic injuring the road.

In practicing this process the times, temperatures and proportions herein disclosed may be varied according to the exact 105 nature of the rock asphalt, the moisture it contains, the quality of its bituminous binder, the size of the mineral aggregate and the exact nature of the bituminous fortifying material. From the above disclosure 110 however the process may be readily applied by those skilled in the art to all grades of rock asphalt and I desire to be limited only by the ensuing claims.

Having described my invention, I claim: 115

1. The process of making roads out of natural rock asphalt, the bituminous content of which is below specifications, comprising the steps of grinding up the natural rock asphalt, heating the same to a temperature 120 of between 100° and 150° F., adding thereto and mixing therewith a predetermined quantity of fortifying bituminous material heated to from 200° to 250° F., applying the resulting material in cold condition to 125 the road to be paved, and exposing the same to action of the sunlight to harden it into a solid mass.

2. The process of fortifying natural rock asphalt with bituminous material compris- 130

ing the steps of grinding the rock asphalt, heating the same to a degree sufficiently hot not to chill unduly the fortifying bitumen and yet not hot enough to cause the mass 5 to set up, adding to and mixing therewith fortifying bitumen heated to a degree sufficient to render the same fluid, and yet not sufficiently hot to cause the bitumen of the rock asphalt to set up.

10 3. The process of fortifying natural rock asphalt with bituminous material without injuring the shipping qualities of the product comprising the step of mixing the natural rock asphalt with the fortifying 15 bituminous material, the temperature of the fortifying bituminous material being such that it is sufficiently fluid to mix readily with the rock asphalt, the temperature of the rock asphalt being such that it will not chill the 20 bituminous material to an extent sufficient to prevent the mixing therewith, the temperature of the entire mass being such that the bituminous binder thereof will not set 25 up and cause the rock asphalt to form a solid rock like mass.

4. The process of fortifying natural rock

asphalt with bituminous material comprising the step of mixing the natural rock asphalt with the fortifying bituminous material, the temperature of the fortifying bituminous material being between 200° and 250° F., and the temperature of the rock asphalt being between 100° and 150° F.

5. The process of making roads out of natural rock asphalt, the bituminous content 30 of which is below specifications comprising the steps of grinding up the natural rock asphalt, heating the same to a temperature slightly below that at which the particular grade of rock asphalt changes in color from 35 gray or brown to black, adding thereto and mixing therewith a predetermined quantity of bituminous material heated to a temperature at which it is sufficiently fluid to mix with the rock asphalt, and applying the 40 resulting gray or brown material in cold condition to the road to be paved, and exposing the same to action of the sunlight 45 preparatory to opening the road to traffic.

In witness whereof, I hereunto subscribe 50 my name.

CHARLTON WILDER.